

## UNITED STATES PATENT OFFICE.

FRANCIS M. ROGERS, OF WHITING, INDIANA, ASSIGNOR TO STANDARD OIL COMPANY,  
OF WHITING, INDIANA, A CORPORATION OF INDIANA.

## TREATING HYDROCARBON OIL RESIDUES.

No Drawing.

Application filed August 28, 1922. Serial No. 584,863.

The present invention relates to improvements in the art of handling heavy residues resulting from a substantially non-cracking distillation of crude, asphalt-bearing petroleum oils.

The residues which are treated in accordance with the present invention are the products resulting when a crude asphalt-bearing petroleum oil, for example, of the character of mid-continent crude oil, is reduced to a bottom or residue having substantially the flash and fire test of the end product desired, the distillation being conducted either with steam or under vacuum so that substantially no cracking has taken place.

In accordance with the present invention, such a residue is mixed with a suitable hydrocarbon oil of lower viscosity, for example, a light paraffin oil or less viscous oil, such as gas oil, kerosene oil or gasoline, the liquid oil mixture being then subjected to treatment with sulfuric acid, for example, of 66° Baumé. The treatment is carried out in accordance with the nature of the final product described, particularly with reference to its color and freedom from asphalt.

After the treatment with acid, the diluent is removed from the oil by substantially non-cracking distillation. After the diluent has been removed, the further treatment of the oil may be varied in accordance with the character of the product desired. For example, the treated oil may be dissolved in naphtha and filtered through fuller's earth or other clarifying material to produce a filtered stock, or may be diluted with naphtha or other suitable solvents, chilled and settled for the removal of petrolatum, a very high flash point bright stock being thereby produced. The reduced oils produced by the treatment are valuable heavy lubricants, cylinder oils, etc. The process is particularly advantageous in connection with residues from asphalt-bearing crude oils representing 10% or less of the volume of the oil.

The following example illustrates the practice of the present invention:

A mid-continent crude oil was reduced with fire and steam to a residuum of about

7%. This residuum is an asphalt having a 50 melting point of about 110° and a penetration at 77° of about 200. A mixture was made containing 30% of this residuum and 70% of miner's oil distillate, the mixture being treated with from 1 to 1½ lbs. of 66° 55 Baumé sulfuric acid per gallon. The treatment is preferably carried out in two or three dumps with removal of sludge after each dump and the resulting sour oil is washed and neutralized. The treated mixture is then subjected to fire and steam distillation to remove the diluent, that is, the miner's oil distillate, and the resulting residual oil was found to have a gravity of 19.8° 60 Baumé, a flash point of 515° F., a pour test 65 of 38° F. and a viscosity of 320 seconds Saybolt at 210° F. The diluent distilled from the oil is saved and is used for admixture with additional residue for subsequent treatment. By such re-use of the diluent, the 70 losses due to treating with sulfuric acid are materially reduced.

The further treatment of the residual oil is determined by the nature of the product desired. If a filtered stock is desired, the 75 oil is dissolved in naphtha and filtered through fuller's earth, a sufficient amount of the latter being used to produce the desired color. If it is desired to reduce the pour test of the oil or to produce a bright stock, 80 it is diluted with naphtha, chilled and settled for a sufficient period of time for the precipitation of the petrolatum contained therein. In either case, the further treatment or finishing of the stock is carried out 85 while it is diluted with naphtha, or other oil-solvent diluent. If naphtha or an equivalent solvent has been employed as the diluent for the pitch residue during the acid treating step, the finishing step, either filtration or chilling and settling, may be carried out prior to the removal of the diluent.

I claim:

1. The method of handling a normally solid, asphalt-like residue obtained by distillation from an asphalt-bearing crude oil substantially without cracking which consists in mixing the residue with a hydrocar-

bon oil of lower viscosity, treating the mixture with sulfuric acid, and removing the admixed hydrocarbon oil from the treated residue.

5. 2. The method of handling a normally solid, asphalt-like residue obtained by distillation from an asphalt-bearing crude oil sub-

stantially without cracking which consists in mixing the residue with acid-treated hydrocarbon oil of lower viscosity, treating the mixture with sulfuric acid and removing the admixed oil from the treated residue. 10

FRANCIS M. ROGERS.